

## UNITED STATES PATENT OFFICE

2,348,317

## LUBRICANT CONTAINING METAL COMPOUNDS

Stanley P. Waugh, Westfield, N. J., assignor to  
Tide Water Associated Oil Company, Bayonne,  
N. J., a corporation of Delaware

No Drawing. Application May 22, 1941,  
Serial No. 394,622

16 Claims.

(Cl. 252—48)

This invention relates to improved mineral oil lubricant compositions, and more particularly to improvements in the type of compositions known as extreme pressure lubricants.

For the past several years the tendency in automotive design has been toward engines of increased power. This and other factors have resulted in operation of automobiles at higher and more sustained speeds. In such operation the bearing surfaces of gears such as transmission and differential gears of the modern automobile are subjected to extremely high unit pressures in operation. This is particularly true in the case of differential gears of the hypoid type now commonly used.

It is well known in the automotive art that the ordinary mineral oil lubricants formerly employed do not adequately lubricate such gears under these high pressure conditions, and this situation has given rise to the development of gear lubricating compositions known in the art as extreme pressure or E. P. lubricants.

The conventional E. P. lubricants comprise a suitable mineral oil and an additional substance which imparts to the composition high load-carrying capacity. In most types of E. P. lubricants which have been proposed the additional substance or E. P. agent, as it is termed, is either sulfur in the free or combined state, or certain chlorine compounds, or both sulfur and chlorine which may be in combination, for example as sulfur chloride.

One requirement of E. P. lubricants is that the E. P. agent therein be of chemically reactive nature since the lubricating effectiveness of these compositions is apparently due to the deposition upon the bearing surfaces of a high load-carrying film produced by chemical reaction involving the E. P. agent. The lubricating effectiveness of E. P. lubricants is thus not due to the viscosity and other characteristics of the mineral oil as in the case of the formerly used gear lubricants containing no E. P. agent, but is essentially attributable to the high load-carrying chemical film.

Although some of the various extreme pressure lubricants heretofore proposed have proved successful for certain uses, a great many have not been satisfactory, particularly for the lubrication of hypoid gears in automobiles and other automotive gears operating under particularly high pressure conditions, mainly because the additive agent fails to impart sufficiently high load-carrying capacity to the compositions, and for other reasons. For example, it is known that the in-

corporation of free sulfur in mineral oils increases the load-carrying capacity over that of the mineral oil alone, but many such compositions fall far short of being satisfactory lubricants for hypoid gears and others under modern high-pressure operating conditions in respect to load-carrying capacity, and for the additional reason that such compositions tend to cause objectionable corrosion of the gear tooth surfaces.

10 Likewise, certain chlorine compounds and sulfur compounds provide some improvement in load-carrying capacity but are insufficiently effective in this and other respects as E. P. ingredients for use in lubricants intended for the stated services.

The present invention provides improved lubricant compositions suitable and effective for the lubrication of bearing surfaces operating under extremely high unit pressures. In one aspect the invention provides a means for increasing the E. P. properties and other desirable characteristics of lubricant compositions of the type normally considered effective to some extent as extreme pressure lubricants for certain lubrication services.

I have found in accordance with this invention that compounds of antimony or bismuth are capable of "activating" or promoting extreme pressure properties of many substances and that by incorporating said metal compounds with said substances improved E. P. lubricant compositions result. By this means the load-carrying capacity of free sulfur-containing mineral oils, for example, can be increased from a point which as stated hereinabove is unsatisfactory for lubrication of hypoid gears and the like to a load-carrying capacity very satisfactory for this purpose. The effectiveness in this respect of sulfur compounds, 30 chlorine compounds such, for instance, as those mentioned hereinabove, and others can be likewise improved by incorporation of such metal compounds. Furthermore, the load-carrying capacities of certain initially effective E. P. lubricant compositions can be improved by incorporation of such metal compounds therein to thus provide a higher safety factor or assured effectiveness to meet future lubrication demands as respects higher unit pressures between bearing surfaces to anticipate future use in the automotive field of engines of increased power.

As agents for use as "activators" or promoters of E. P. properties when incorporated according to this invention, I have found that both organic and inorganic compounds of antimony and

bismuth are suitable. Halides, such for example as antimony trichloride, and alcoholates such for example as antimony or bismuth iso-amylates or ethylates, have proved particularly suitable. Likewise cyclic or aromatic derivatives are effective, examples of these being aromatic stibines or bismuthines, for example triphenyl stibines and triphenyl bismuthines. Soaps of such metals are also satisfactory. Among the latter class may be named soaps of cyclic nature such as naphthenates, for example antimony naphthenates, or soaps of aliphatic straight chain acids. Antimony oleate may be mentioned as representative of the latter class. In general, however, the metal soaps of the straight chain aliphatic acids are less effective than the other metal compounds discussed hereinabove.

The invention, broadly stated, comprises lubricant compositions containing E. P. agents and having incorporated therein one or more metal compounds of the class described hereinabove which is effective to promote or increase the load-carrying capacity of said agent.

The exact reason why the addition of the described metal compounds improves the load-carrying capacity of these compositions is not known. The improvement cannot be attributed to an additive effect, inasmuch as the metal compounds themselves have no appreciable E. P. properties. In other words, the load-carrying capacity of a given lubricant composition of this invention containing say free sulfur and antimony trichloride will be very much greater than the sum of the respective load-carrying capacities of the sulfur and the antimony trichloride.

The lubricant compositions of the invention may be prepared in any suitable manner. The metal compound to be used as the promoter may be simply stirred into a suitable mineral oil containing the agent the E. P. property of which is to be improved or the metal compound may be dissolved in mineral oil and the resulting mixture added to the said agent. Mixing may be carried out at normal room temperatures, or, if desired, with heating, care being taken, however, not to heat to temperatures at which chemical reaction destructive to the desired properties of the composition occurs. For example, in the case of mineral oil containing sulfur in which antimony has been incorporated, heating to temperatures of around 180° F. or above may cause precipitation of antimony sulfide, thus removing from solution important substances. Ordinarily temperatures up to about 150-160° F. may be used in this instance.

The antimony or bismuth compounds are effective in relatively small amounts, generally in proportions of about 10% or less on the basis of the whole composition and proportional amounts of about 1% have been found suitable in most cases. In the case of soaps of these metals, however, it has been found that in some instances more is required to obtain satisfactory results than is required of other metal compounds. Antimony soaps, for example, should be added in minimum proportions of from about 5% to about 10% of the total composition.

In order to evaluate the working strength or load-carrying capacity of lubricants prepared in accordance with the instant invention such lubricants were tested on the S. A. E. lubricants' tester. This machine is described in detail in S. A. E. Journal, July 1936, page 293. It affords a recognized and standardized test for determination of actual load-carrying capacities of E. P. lubri-

cants. Briefly, the machine comprises two rotatable hardened steel test rings rotated in opposite directions against each other so as to make theoretical line contact at their peripheries. The rings are rotated one clockwise at 890 R. P. M. and the other counter-clockwise, the speed ratio being 14.6 to 1, and a lever mechanism is provided for increasing the force between the bearing surfaces of the rings at a definite loading rate. The mechanical advantage of the lever is about 10 to 1 and a scale is provided which indicates in pounds (up to 600 pounds) the force applied to the lever. The oil to be tested is continuously supplied at the rubbing-rolling surface at which the rings form mutual contact.

The pressure at which a given oil fails in this test is indicated by the scale reading at the time when sparking occurs between the adjacent ring surfaces. Sparking indicates that the ring surfaces have become scored or scuffed and this may be substantiated by subsequent inspection.

In the following tests on the S. A. E. tester the loading rate (scale) was 83.5 lbs./sec.

Numerous lubricating compositions prepared in accordance with the present invention were tested on this machine. In these tests the following two blends of mineral oil were employed as the lubricant base for the indicated assistant and promoter:

- 30 1. { 56% steam refined cylinder stock  
44% pale oil  
2. { 33% pale oil  
67% bright stock

35 In these blends, the cylinder stock used was an unfiltered residual oil having a Saybolt viscosity at 210° F. of about 180 seconds, the bright stock a filtered residual stock derived from a Pennsylvania crude having a Saybolt viscosity at 210° F. of approximately 150 seconds, and the pale oil a light-colored filtered oil having a Saybolt viscosity at 100° F. of approximately 200 seconds, derived as an overhead cut from a non-Pennsylvania crude. A third blend comprising heavy red oil, derived as distillate from a Columbian crude, and pale oil was also used in some of the tests as will appear.

40 It is, of course, understood that these blends were selected merely as convenient oils for blending in suitable proportions to obtain whatever viscosity is desired in the finished lubricant. Other stocks could be substituted without affecting the ultimate result.

45 In some of the tests, as will be apparent, the lubricant was first subjected to a heat test wherein the lubricant was heated for a period of 16 hours at 180° F. prior to the test on the S. A. E. lubricants' tester. In other tests, where indicated, the lubricant was first subjected to a more severe heat test wherein said lubricant was heated at a temperature of 200° F. for 84 hours prior to the S. A. E. test.

50 In the following tests of examples of lubricating compositions of the invention all withstood the maximum load of the S. A. E. machine as indicated by the fact that the maximum scale reading was reached without failure or reduction in effectiveness of the lubricants.

- 55 1. { 56% steam refined cylinder stock  
95% { 99% { 56% steam refined cylinder stock  
1% added sulfur  
5% antimony isoamylate  
2. 50% above composition  
50% sulfurized mineral oil

|     |                                                                                                                                                              |     |                                                                                                                                                                                                                                                                                                                                                                                                                                                                                                                                                                                                                                                                                                                                                                                                                                                                                                                                                              |
|-----|--------------------------------------------------------------------------------------------------------------------------------------------------------------|-----|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 2.  | 90% { 56% steam refined cylinder stock<br>90% { 44% pale oil<br>1% added sulfur<br>1% antimony isoamylate                                                    | 20. | 94% { 56% steam refined cylinder stock<br>94% { 44% pale oil<br>1% added sulfur<br>5% bismuth isoamylate                                                                                                                                                                                                                                                                                                                                                                                                                                                                                                                                                                                                                                                                                                                                                                                                                                                     |
| 4.  | 90% { 33% pale oil<br>90% { 67% bright stock<br>1% added sulfur<br>2% antimony isoamylate                                                                    | 5.  | The following test data from tests made on the S. A. E. tester under the same test conditions as described hereinabove upon compositions similar to those described but containing none of the metal compounds of this invention afford comparisons which bring out the effect of the additive activator or promoter agents:                                                                                                                                                                                                                                                                                                                                                                                                                                                                                                                                                                                                                                 |
| 5.  | 90% { 33% pale oil<br>97.2% { 90% { 67% bright stock<br>1% added sulfur<br>2.0% antimony isoamylate<br>0.8% oleic acid                                       | 10. | 21. 56% steam refined cylinder stock Failed at 40-60 pounds S. A. E. tester scale reading<br>44% pale oil                                                                                                                                                                                                                                                                                                                                                                                                                                                                                                                                                                                                                                                                                                                                                                                                                                                    |
| 6.  | 90% { 56% steam refined cylinder stock<br>96% { 44% pale oil<br>1% added sulfur<br>2% antimony isoamylate<br>2% oleic acid                                   | 15. | 22. 90% of No. 21 blend Failed at 150 pounds S. A. E. tester scale reading<br>10% chlorinated wax                                                                                                                                                                                                                                                                                                                                                                                                                                                                                                                                                                                                                                                                                                                                                                                                                                                            |
| 7.  | 90% { 56% steam refined cylinder stock<br>96% { 44% pale oil<br>1% added sulfur<br>2% oleic acid<br>2% antimony ethylate                                     | 20. | 23. 90% of No. 21 blend Failed at 250 pounds S. A. E. tester scale reading<br>1% added sulfur                                                                                                                                                                                                                                                                                                                                                                                                                                                                                                                                                                                                                                                                                                                                                                                                                                                                |
| 8.  | 90% { 56% steam refined cylinder stock<br>98% { 44% pale oil<br>10% chlorinated wax<br>2% antimony isoamylate                                                | 25. | 24. 80% of No. 21 blend Failed at 210 pounds S. A. E. tester scale reading<br>20% corn oil, 10% sulfurized                                                                                                                                                                                                                                                                                                                                                                                                                                                                                                                                                                                                                                                                                                                                                                                                                                                   |
| 9.  | 90% { 56% steam refined cylinder stock<br>97% { 80% { 44% pale oil<br>20% sulfurized corn oil (non-corrosive)<br>3% antimony isoamylate                      | 30. | The fact that the lubricant compositions of the instant invention withstand the maximum load on the S. A. E. tester indicates them to have outstanding load-carrying properties. Although it was impossible to determine the exact load at which these compositions would fail, due to the limits of the testing machine, the condition of the test ring surfaces after the tests indicated that even considerably higher loads would not cause failure. The surfaces of the used test rings were unusually smooth in contrast to surfaces of other rings which had been used in testing certain other good E. P. lubricants. The rings showed substantially no signs of wear and no evidence of scuffing or scoring.                                                                                                                                                                                                                                        |
| 10. | 90% { 56% steam refined cylinder stock<br>96% { 44% pale oil<br>1% added sulfur<br>2% tetrachlorophenyl ether<br>2% Sb isoamylate                            | 35. | 35. An additional advantageous feature of the compositions of the invention resides in the fact that the added metal compounds described also function to inhibit corrosion of metal surfaces of parts being lubricated by the composition. This is evidenced by the bright condition of the S. A. E. machine test rings used in testing these lubricants. These rings showed no evidence of pitting or undue chemical attack after use in the test. Thus, use of the lubricants of this invention in heavy duty gear lubrication will result in prolonged gear life in protecting the bearing surfaces thereof from undesirable chemical attack as well as from rapid physical wear. Certain substances heretofore used as E. P. ingredients which normally are of such high chemical activity as to cause undesirable corrosion may be stabilized or inhibited in this respect by incorporation of the described metal compounds.                          |
| 11. | 90% { 56% steam refined cylinder stock<br>98% { 95% { 99.5% { 44% pale oil<br>0.5% added sulfur<br>5% chlorinated wax<br>2% antimony isoamylate              | 40. | 40. The described metal compounds are desirably employed in solution in the mineral oil component, but need not be dissolved since they function in suspension as well. Metal compounds of the stated class which are substantially oil-insoluble may if desired be rendered soluble by first dissolving them in certain other substances. For example, in preparing compositions numbered 18 and 19 hereinabove the antimony trichloride was first dissolved in peanut oil and palm oil respectively, and these mixtures were added to the mineral oil blends shown. Other solubilizing agents found effective, particularly for antimony compounds, are certain wood fatty acids and certain phosphate esters such, for example, as lauryl phosphate. In some of the compositions, when allowed to stand for several hours, a slight sediment may form. This, however, in no way detracts from the effectiveness of the composition as an E. P. lubricant. |
| 12. | 90% { 56% steam refined cylinder stock<br>98% { 90% { 44% pale oil<br>7% chlorinated wax<br>3% sulfurized corn oil (non-corrosive)<br>2% antimony isoamylate | 45. | 45. Likewise, the alcoholates of the described metals may be stabilized, the use of fatty acids                                                                                                                                                                                                                                                                                                                                                                                                                                                                                                                                                                                                                                                                                                                                                                                                                                                              |
| 13. | 90% { 56% steam refined cylinder stock<br>96% { 44% pale oil<br>10% chlorinated wax<br>2% antimony isobutyrate                                               | 50. |                                                                                                                                                                                                                                                                                                                                                                                                                                                                                                                                                                                                                                                                                                                                                                                                                                                                                                                                                              |
| 14. | 90% { 56% steam refined cylinder stock<br>99% { 44% pale oil<br>1% added sulfur<br>10% Sb naphthenate                                                        | 55. |                                                                                                                                                                                                                                                                                                                                                                                                                                                                                                                                                                                                                                                                                                                                                                                                                                                                                                                                                              |
| 15. | 90% { 56% steam refined cylinder stock<br>95% { 99% { 44% pale oil<br>1% added sulfur<br>5% Sb naphthenate                                                   | 60. |                                                                                                                                                                                                                                                                                                                                                                                                                                                                                                                                                                                                                                                                                                                                                                                                                                                                                                                                                              |
| 16. | 90% { 56% steam refined cylinder stock<br>90% { 44% pale oil<br>1% added sulfur<br>10% Sb oleate                                                             | 65. |                                                                                                                                                                                                                                                                                                                                                                                                                                                                                                                                                                                                                                                                                                                                                                                                                                                                                                                                                              |
| 17. | 92% { 56% steam refined cylinder stock<br>92% { 44% pale oil<br>1% added sulfur<br>8% Base { 80% mineral oil<br>20% triphenylstibine                         | 70. |                                                                                                                                                                                                                                                                                                                                                                                                                                                                                                                                                                                                                                                                                                                                                                                                                                                                                                                                                              |
| 18. | 90.15% { 90% heavy red oil<br>90% { 0.85% added sulfur<br>10% SbCl <sub>3</sub> solution { 10% SbCl <sub>3</sub><br>10% peanut oil                           | 75. |                                                                                                                                                                                                                                                                                                                                                                                                                                                                                                                                                                                                                                                                                                                                                                                                                                                                                                                                                              |
| 19. | 90.15% { 90% heavy red oil<br>90% { 0.85% added sulfur<br>10% SbCl <sub>3</sub> solution { 10% SbCl <sub>3</sub><br>10% palm oil                             |     |                                                                                                                                                                                                                                                                                                                                                                                                                                                                                                                                                                                                                                                                                                                                                                                                                                                                                                                                                              |

being particularly advantageous for the purpose. Oleic acid, for example, functions in the sulfur compositions (see Formulae 5, 6 and 7) to stabilize the antimony alcoholates against hydrolyzation, thus preventing precipitation of antimony sulfide which may normally occur under high temperature conditions, such, for example, as is encountered in the heat tests of Examples 6 and 7. The presence of oleic acid does not reduce the load-carrying capacities of the compositions, which is surprising in view of the fact that the normal effect of oleic acid in E. P. lubricants is to reduce load-carrying capacity.

In addition to gear lubricants the invention is also applicable to various other types of lubricants. For example, cutting oils and the like for use in extreme pressure metal working operations, and in general all lubricants for use where high bearing pressures exist, are included within the scope of the invention.

The invention also includes methods of lubricating metal surfaces comprising applying thereto the compositions disclosed herein.

I claim:

1. A lubricant composition comprising an E. P. agent and chlorinated materials selected from the group consisting of sulfur, sulfurized materials and a compound of a metal of the group consisting of antimony and bismuth per se possessing no appreciable E. P. properties but being effective to enhance the load-carrying capacity of said E. P. agent, the metal in said compound being in the monoatomic form.

2. A lubricant composition comprising mineral oil, an agent having load-carrying capacity selected from the group consisting of sulfur- sulfurized materials and chlorinated materials and a compound of a metal of the group consisting of antimony and bismuth per se possessing no appreciable load-carrying capacity but being effective to enhance the load-carrying capacity of said agent, the metal in said compound being in the monoatomic form.

3. An extreme pressure lubricant composition comprising mineral oil and a substance normally having low load-carrying capacity selected from the group consisting of sulfur, sulfurized materials and chlorinated materials and a compound of the group consisting of antimony and bismuth per se possessing no appreciable load-carrying capacity, but being effective to enhance the load-carrying capacity of said substance, the metal in said compound being in the monoatomic form.

4. A lubricant composition comprising a chlorinated material and a compound of a metal selected from the group consisting of antimony and bismuth effective to increase load-carrying capacity of said chlorine-containing compound.

5. A lubricant composition comprising mineral oil, sulfur and a compound of a metal of the group consisting of antimony and bismuth per se possessing no appreciable load-carrying capacity but being effective to increase the load-carrying capacity of the sulfur, the metal in said compound being in the monoatomic form.

6. An extreme pressure lubricant composition comprising mineral oil, sulfur and an antimony

soap effective to increase the load-carrying capacity of the sulfur.

7. A lubricant composition comprising an E. P. agent selected from the group consisting of sulfur, sulfurized materials and chlorinated materials and an alcoholate of a metal selected from the group consisting of antimony and bismuth effective to enhance the load-carrying capacity of said E. P. agent.

10 8. A lubricant composition comprising a mineral lubricating oil, sulfur and an alcoholate of a metal selected from the group consisting of antimony and bismuth, said alcoholate being present in an amount sufficient to enhance the load-carrying property of the sulfur.

15 9. A lubricant composition comprising a mineral lubricating oil, sulfur and a compound selected from the group consisting of antimony isoamylate and bismuth isoamylate, said compound being present in an amount sufficient to enhance the load-carrying property of the sulfur.

20 10. A lubricant composition comprising a mineral lubricating oil, a substance having load-carrying capacity selected from the group consisting of sulfur, sulfurized materials and chlorinated materials, and a compound of a metal selected from the group consisting of antimony and bismuth per se possessing no appreciable load-carrying capacity but being effective to enhance the load-carrying properties of the substance of the first named group, the metal in said compound being in the monoatomic form.

25 11. A lubricant composition comprising a mineral oil having dissolved therein sulfur and antimony chloride, said antimony chloride being present in an amount sufficient to enhance the load-carrying property of the sulfur.

30 12. A lubricant composition comprising a mineral oil containing sulfur, having dissolved therein antimony chloride and an agent effective to stabilize the antimony chloride, said antimony chloride being present in an amount sufficient to enhance the load-carrying property of the sulfur.

35 13. A lubricant composition comprising a sulfur-containing mineral oil having dissolved therein antimony chloride and a vegetable oil effective to stabilize the solution, said antimony chloride being present in an amount sufficient to enhance the load-carrying property of the sulfur.

40 14. An extreme pressure lubricant composition comprising a mineral oil having dissolved therein sulfur, an antimony alcoholate and a fatty acid effective to stabilize the solution, said antimony alcoholate being present in an amount sufficient to enhance the load-carrying property of the sulfur.

45 15. An extreme pressure lubricant composition as described in claim 14, in which the fatty acid is oleic acid.

50 16. An extreme pressure lubricant composition comprising mineral oil, a load-carrying agent selected from the group consisting of sulfur, sulfurized materials and chlorinated materials, and a stibine effective to enhance the load-carrying properties of said agent.

STANLEY P. WAUGH.